

A. L. J. QUENEAU.  
METALLURGY OF ZINC.  
APPLICATION FILED DEC. 17, 1908.

1,114,036.

Patented Oct. 20, 1914.



WITNESSES:

M. A. Rice  
H. Johnson

INVENTOR:  
A. L. J. Queneau,  
BY  
Leanne & Goldsborough,  
ATTORNEYS

# UNITED STATES PATENT OFFICE.

AUGUSTIN LÉON JEAN QUENEAU, OF TORRESDALE, PENNSYLVANIA, ASSIGNOR TO QUENEAU ELECTRIC ZINC FURNACE COMPANY, OF PHILADELPHIA, PENNSYLVANIA, A CORPORATION OF DELAWARE,

## METALLURGY OF ZINC.

1,114,036.

Specification of Letters Patent. Patented Oct. 20, 1914.

Application filed December 17, 1908. Serial No. 467,986.

To all whom it may concern:

Be it known that I, AUGUSTIN LÉON JEAN QUENEAU, a citizen of the Republic of France, residing at Torresdale, county of Philadelphia, and State of Pennsylvania, have invented certain new and useful Improvements in Metallurgy of Zinc; and I do hereby declare the following to be a full, clear, and exact description of the invention, such as will enable others skilled in the art to which it appertains to make and use the same.

The standard practice of today in the smelting of zinc ores is to roast the ores to remove the sulfur from the sulfid ores or the carbon dioxide from the carbonates. The resulting zinc oxid mixed with finely divided coal is reduced in small fire clay retorts (holding from 50 to 150 pounds of charge) fitted up in tiers within a heated furnace, the heat passing through the wall of the retorts. The zinc vapors issue into short fire clay receivers where they condense into molten metal. That this process is an extremely inefficient one has long been recognized, but the many attempts to supplant it have heretofore been unsuccessful. The inefficiency of the process arises from the fact that the ore mixture must be heated to about 1200 degrees C. Consequently, the retorts must have thin walls, in order to transmit to the charge the heat required, and must be made of fire clay which alone possesses the necessary plasticity for the purpose. The fire clay retorts are difficult to make, fragile, readily attacked by slag, and absorb considerable quantities of zinc, which is lost when the retorts are destroyed. The heat efficiency is very low and the average life of the retorts hardly more than thirty days. The condensation of the zinc vapor also presents difficulties, and much of it is collected as a metallic powder which must be re-distilled, in order to be condensed to the liquid state.

In contrast to the standard practice above indicated, the present invention permits the treatment of the ores in receptacles of large size, adapted to contain a correspondingly large charge. Furthermore, it permits the thickness of the walls of the containing ves-

sel to be greatly increased and permits them to be made of a material more resistant to the action of slag than fire clay. Moreover, in the treatment of zinc ores containing sulfur it is not necessary, in order to adapt them to the uses of the invention, that they should first be brought to a sweet roast, inasmuch as the reduction of the ores by means of iron, or by means of lime and carbon, according to the formulae



and



can be readily effected, particularly in view of the fact that during the reducing operation, the reducing agents are brought into intimate contact with the ore. It is, therefore, desirable merely to roast the zinc sulfid ores to a sulfur content of five or six per cent., which can be brought about with a small expenditure of coal, and, in fact, zinc ores in the raw or unroasted condition may be treated in accordance with the invention. Furthermore, in the practice of the invention, zinc ores carrying copper, lead, iron, gold or silver can be commercially treated, and to particular advantage if to the zinc ores carrying gold or silver, some copper ore is added to form a copper matte to take up the precious metals.

In the present practice the employment of ores high in slag-forming elements corrosive to the fire clay walls of the retorts is avoided, as it is necessary to have the reduction residues present in a dry pulverulent condition in order to allow of their easy removal from the retorts, and for this reason a large excess of reducing material is used to act as a sponge, holding apart any slag-forming material. On the other hand, as will appear from the description of the furnace, in the present instance, it is necessary to have the residual products of the treated charge in a highly fluid state and of a chemical composition having the minimum dissolving power for zinc compounds. It follows, therefore, that ores that are of an objectionable chemical composition for the present practice but which are of low cost are highly desirable for the practice of the

present invention. In the practice of the invention it is also feasible to pre-heat the ore to a high temperature before admitting it into the reduction furnace, for instance, to pre-heat it to a temperature of say 1000° C. This pre-heating of the ore may be attained in the ordinary roasting kilns, and is incident to the roasting of the ores in such kilns; so that the ore, after its sulfur content is reduced to the low limit incident to the roasting operation and is discharged from the kiln, may be discharged directly into the zinc-reducing furnace, or may be temporarily stored in a receptacle which will conserve or substantially conserve the high heat of the ore until the zinc-reducing furnace is ready to receive it. Whether the high preliminary heat of the ore is an incident of the roasting operation or is otherwise imparted to it, such temperature is higher than the temperature at which the coal or other reducing agent would burn in the air. For this reason, the mixing of the reducing agent with the ore should preferably take place within the furnace itself. Nevertheless, it will be found of advantage to also pre-heat the reducing agent, but at a temperature lower than that at which it would burn in the air, the ore and the reducing agent being charged separately into the reducing furnace and mixed therein by revolving the latter.

In carrying out the invention, it will be desirable to heat the interior of the rotary reduction furnace to a high temperature, by a gas and air flame, or the like, before admitting the furnace charge. To then maintain the reducing temperature during the subsequent reduction of the ore and distillation of the zinc therefrom a molten fluid resistor is employed, which is introduced into the furnace chamber, in such manner as to form a path for an electric current of such a character as to maintain the fluidity of the resistor and the high temperature necessary to carry on and complete the reducing operation, the surfaces of contact between the charge and the fluid resistor being constantly renewed by reason of the rotative movement of the furnace chamber, thereby increasing the speed of the reaction. The zinc vapors given off by the charge are received in condensers of such construction and arrangement that the vapors are condensed therein to the metallic liquid state, special provision being made for regulating and maintaining the temperature conditions desirable for the recovery of the zinc in this form.

A furnace suitable for the purposes of the invention is illustrated in United States Letters Patent No. 1,006,876, granted to me under date of October 24, 1911, and I refer specifically thereto for the details of con-

struction and the mode of operation appropriate to such a furnace.

In the drawing, hereunto attached, I have illustrated diagrammatically the general assemblage of apparatus of which the furnace referred to, or its equivalent, forms a constituent part.

In this drawing, A indicates the zinc ore preheater, B represents the reducing furnace receiving its charge of zinc ore from the preheater, and C indicates a condenser. The reducing agent is charged into the reducing furnace preferably from a preheater as indicated at D, and the furnace and condenser are preferably of the rotary type as indicated.

Speaking further of the general operation of the invention, it will be noted that the agitation of the contents of the furnace, due to the rotation, results in close and intimate contact between the constituents of the furnace charge, thereby shortening the time required for the complete chemical action, and not only increasing the daily furnace capacity, but also increasing the heat efficiency of the furnace, as heat is radiated, for a given charge, during a shorter space of time, so that the loss of radiated heat is correspondingly less. Furthermore, the rotation and agitation of the contents of the furnace result in the rapid attainment of an equilibrium of temperature throughout the mass of the charge, and the rotation of the furnace, by constantly renewing the surface of the lining in contact with the heating medium, keeps the whole furnace at a high heat. Evidently, however, the upper part of the furnace will be at all times to some extent cooler than the lower part which contains the molten resistor. This is a desirable feature, in that it keeps at a minimum the temperature of the issuing gases and vapors, thus facilitating the condensation of the latter while keeping at a minimum the number of heat units carried away by the gases.

What I claim is:—

1. The method of extracting and recovering zinc from zinc ore, which consists in pre-heating said zinc ore, separately charging into a reducing furnace the ore in the pre-heated state and a reducing agent, intimately mixing them within the furnace, subjecting the mixture to a reducing atmosphere and a reducing temperature with exclusion of air, thereby releasing the zinc in the form of zinc vapor, and condensing said vapor to the metallic state.

2. The method of extracting and recovering zinc from zinc ore, which consists in preheating said zinc ore to a temperature above that at which the reducing agent to be used would burn in air, separately charging into a reducing furnace the ore in the

preheated state and a reducing agent, intimately mixing them within the furnace, subjecting the mixture to a reducing atmosphere and a reducing temperature with exclusion of air, thereby releasing the zinc in the form of zinc vapor, and condensing said vapor to the metallic state.

In testimony whereof I affix my signature, in presence of two witnesses.

AUGUSTIN LÉON JEAN QUENEAU.

Witnesses:

JOHN C. PENNIE,

LAURA B. PENFIELD.